

## UNITED STATES PATENT OFFICE.

DANIEL H. MELOCHE, OF DETROIT, MICHIGAN, ASSIGNOR TO EARL HOLLEY, OF DETROIT, MICHIGAN.

## METHOD OF COATING METAL MOLDS.

No Drawing.

Application filed March 14, 1923. Serial No. 625,141.

*To all whom it may concern:*

Be it known that I, DANIEL H. MELOCHE, a citizen of the United States, residing at 2241 Gladstone Ave., Detroit, in the county of Wayne and State of Michigan, have invented certain new and useful Improvements in Methods of Coating Metal Molds, of which the following is a specification.

This invention relates to an improved method of coating metal molds; specifically it refers to an improved method of applying a protective lining to cast iron molds, the lining being adapted to withstand the erosive action of molten metal.

One of the difficulties experienced when it has been heretofore attempted to coat metal molds with a coating sufficiently substantial to withstand the flow of iron was that such a coating would blister and flake off during and after the casting operation. It is the object of this invention to apply a permanent coating which will stand repeated use and be substantially intact after a day's run during which hundreds of castings are cast in the permanent mold.

The method I have discovered consists in first mixing a 10% solution of sodium silicate in water with an equal weight of finely ground fire clay. Then thoroughly mixing the dilute solution of sodium silicate with the powdered fire clay, then heating the cast iron molds which may preferably be made hollow as shown in the co-pending application of Peter W. Mulder, Serial No. 541,288, filed March 6, 1922, to from 300° to 500° F., then applying with a brush the mixture of fire clay and sodium silicate solution. This coating is only a few thousands of an inch in thickness. An air spray may be substituted for the brush.

Immediately after the thin coating of fire clay and soluble silicate coating is applied a

flame of a blow torch is directed against the surface of the freshly painted mold so as to fix or bake the coat and also to raise the 45 temperature of the mold to what it was before it was cooled by the application of the dilute sodium silicate solution.

Another coating of fire clay is applied as before and the heating operation is repeated 50 until the lining is of the desired thickness.

The mold coating of fire clay with sodium silicate binder is described in my co-pending application, Serial No. 581,239, filed August 11, 1922. 55

What I claim is:

1. The method of applying a protective coating to metal molds which consists in first heating the molds to between 300° and 500° F., then painting the heated surface of the molds with a wash containing a little soluble silicate in solution and a considerable quantity of powdered fire clay in suspension, then heating the surface of the mold, then applying another coat of fire clay with a 60 soluble silicate binder, again heating the surface of the mold and repeating the operation until the desired thickness of fire clay is applied to the surface of the mold.

2. The method of applying a protective 70 coating to metal molds which consists of first mixing a refractory insulating powder with water containing a little heat-resisting binder in solution, then heating the surface of the metal molds to between 300° and 500° F., then painting the surface of the heated metal mold with the said refractory wash, then heating the mold again, then applying another coating of the refractory wash, again heating the mold and repeating until 75 80 a lining of sufficient thickness is obtained.

In testimony whereof I affix my signature.

DANIEL H. MELOCHE.